

Sept. 30, 1952

H. M. HOXIE

2,611,929

METHOD OF PRODUCING SHAPED ARTICLES FROM ARTIFICIAL  
OR SYNTHETIC FIBER OR FILM-FORMING MATERIALS

Filed June 18, 1951



INVENTOR.  
HOWARD M. HOXIE  
BY

*Thomas B. McAllister*  
ATTORNEY.

## UNITED STATES PATENT OFFICE

2,611,929

METHOD OF PRODUCING SHAPED ARTICLES  
FROM ARTIFICIAL OR SYNTHETIC FIBER-  
OR FILM-FORMING MATERIALSHoward M. Hoxie, Chester, Pa., assignor, by mesne  
assignments, to The Chemstrand Corporation,  
Decatur, Ala., a corporation of Delaware

Application June 18, 1951, Serial No. 232,208

14 Claims. (Cl. 18—54)

1

This invention relates to improvements in the production of synthetic or artificial fibers, films, or other shaped articles by the wet-spinning or wet-forming processes.

This application is a continuation-in-part of my application Serial No. 125,679 filed November 5, 1949, issued as Patent Number 2,577,763, December 11, 1951.

In wet-spinning or wet-forming, as conventionally practiced, a solution of the material to be shaped is extruded into a vessel containing a suitable setting liquid which is continuously or periodically withdrawn from the vessel, reconditioned, and returned to the extrusion vessel.

In making shaped articles from fiber- or film-forming materials by a wet-spinning or wet-forming process in which chemical reaction is not involved, it has been found advantageous to extrude the solution into a setting medium comprising a controlled, predetermined proportion of the solvent and a precipitant for the fiber-forming material which is an extractive for the extrusion solvent but chemically inert to the fiber- or film-forming material. Thus, in wet-spinning fiber-forming acrylonitrile polymers, improved results are obtained by spinning a dimethylformamide solution of the polymer into a setting bath consisting of water and dimethylformamide in controlled predetermined proportions, as disclosed in my pending application Serial No. 62,413, filed November 27, 1948.

The present invention is concerned more particularly with wet-spinning or wet-forming processes in which a solution or dispersion of the fiber- or film-forming material is extruded into a setting bath comprising the solvent and a precipitant in critical, controlled relative proportions which must be maintained throughout the extrusion, and has as one object to facilitate maintaining the relative proportion of solvent to precipitant in the setting bath substantially constant from the beginning to the end of the extrusion.

In accordance with the invention, a solution or dispersion of the fiber- or film-forming material is extruded into a setting bath comprising the predetermined proportion of solvent and precipitant to form the shaped article, the article is withdrawn from the bath and, prior to any drying thereof, it is washed with the precipitant, or with a mixture of the precipitant and a minor proportion of the solvent, and liquid from this initial washing of the article is continuously delivered to the setting bath. The constituents of the liquid from the washing step

2

are the same as the constituents of the setting bath, and by correlating the proportion of precipitant to solvent in the liquid from the washing and the rate of flow of such liquid into the setting bath with the amount of solvent introduced into the bath by the solution of the material to be shaped, the composition of the bath may be maintained constant. Therefore, when operating in accordance with the invention, it is unnecessary to withdraw the setting bath from the vessel in which the extrusion is performed, or to depend on periodic or hap-hazard additions of either solvent or precipitant to the bath in order to maintain the composition of the bath constant.

The method of the invention can be used for producing artificial or synthetic fibers or other shaped articles from any fiber- or film-forming material which can be dissolved or dispersed and wet-spun, when the shaping involves precipitation only. Examples of suitable fiber- and film-forming materials are the organic acid esters of cellulose, the fiber-forming synthetic resins including polyamides, polyesters, fiber-forming vinyl resins, polyvinyl alcohol, and fiber-forming polymers of acrylonitrile.

The solvent or dispersing agents selected will depend on the particular fiber- or film-forming material to be shaped. As examples of suitable solvents or dispersing agents may be mentioned, acetone for commercial, secondary, cellulose acetate and such fiber-forming vinyl resins as those resulting from the conjoint polymerization of vinyl chloride and vinyl acetate or of vinyl chloride and acrylonitrile and containing from 40 to 55% acrylonitrile in the molecule; hot phenol or formamide for polyamides; chloroform for the polyesters; and dimethylformamide, dimethylacetamide or dimethylpropionamide for acrylonitrile polymers containing from 70 to 98% by weight of acrylonitrile in the molecule and obtained by polymerizing acrylonitrile with one or more other monohylenically unsaturated polymerizable substances including vinyl acetate, styrene, vinyl chloride, vinyl monomers containing basic tertiary nitrogen such as the vinylpyridines and particularly the 2-vinylpyridines, 5-vinyl 2-methylpyridine and the like, isobutene, dimethylfumarate, methylmethacrylate, methacrylonitrile and acrylic acid and its esters. The solvent and dispersing agents mentioned are illustrative only and other solvents or dispersing agents may be substituted for them.

The precipitant selected will depend on both the fiber- or film-forming material being shaped

and the solvent or dispersing agent in which such material is dissolved or dispersed. It may be any liquid which is an extractive for the extrusion solvent or dispersing agent but inert to the fiber-forming material. When water meets this essential requirement, water is the preferred precipitant for use in the setting bath and as the major component of the washing liquid to which the fibers or the like are subjected immediately after their withdrawal from the bath.

A specific embodiment of the invention contemplates the production of fibers or threads from solutions or dispersions of acrylonitrile polymers containing, by weight in the polymer molecule, at least 70% of acrylonitrile, in dimethylacetamide, by spinning the solution into a setting medium consisting of water and a controlled proportion of dimethylacetamide. In a preferred embodiment, a solution of the acrylonitrile polymer in dimethylacetamide is continuously extruded into a setting bath comprising a mixture of water and dimethylacetamide containing the dimethylacetamide in a selected proportion between 20 and 70% by volume, and the composition of the setting bath is maintained constant by washing the fibers as they are withdrawn from the bath with water or water containing a minor proportion of dimethylacetamide, and delivering the liquid from the washing step into the setting bath at a controlled rate. The conditions are selected so that the composition of the setting bath does not vary more than 2% from the predetermined volumetric proportions and the proportion of dimethylacetamide present in the setting bath is at least 20% by volume.

At the start of operations under any given set of spinning conditions, the proportion of precipitant to solvent required in the liquid from the washing step and the rate at which that liquid must be delivered to the setting bath to maintain the composition of the bath constant, can be determined by observation of the refractive index of the bath. Thereafter, adjustments in the washing conditions and in the rate at which the wash liquid is delivered to the bath are generally not required so long as the spinning conditions are not changed. However, if such adjustments are required, they may be made simply by increasing or decreasing the rate of flow of the washing liquid to the washing zone, and/or by increasing or decreasing the rate of flow of the liquid from the washing step to the setting bath. Suitable apparatus for the production of artificial or synthetic fibers or threads in accordance with the invention is illustrated in the accompanying drawing in which the single figure is a diagrammatic, perspective view of a preferred embodiment of the invention.

Referring to the drawing, the solution of the fiber-forming material is extruded through the spinneret 1 into vessel 2 containing a setting bath comprising the predetermined relative proportions of solvent and precipitant. The fibers are withdrawn from the bath under the guide 3 and lapped around godet 4, a thread displacing guide 5 being supported adjacent the godet. From godet 4, the fibers are passed upwardly through the open trough 6 and lapped around godet 7, a thread displacing guide 8 being supported adjacent to that godet to assist in laying the fibers. As shown, godets 4 and 7 are of the same size and may be driven at different peripheral speeds to stretch the fibers. If desired, godets 4 and 7 may be of different sizes and driven at the same speed to accomplish the stretching. As the

fibers advance upwardly through the trough 6, they are washed by liquid supplied to the trough from the vessel 9 with which the trough communicates, for example, with water which may be heated to a temperature up to 100° C., for instance from room temperature to 100° C. The liquid precipitant for the washing, or the mixture of the precipitant with a minor proportion of solvent, is metered into vessel 9 through pipe 10 provided with valve 11, and vessel 9 is provided with a vertically adjustable overflow pipe 12 for adjusting the level of the liquid in vessel 9 to thereby adjust or control the quantity of precipitant or of precipitant-solvent mixture delivered to the trough. The liquid flows downwardly through the trough countercurrently to the direction of the fibers and is collected in the vessel 13 supported adjacent to vessel 2 containing the setting bath. A controlled portion of that liquid, which always comprises a mixture of the precipitant and the solvent, is continuously delivered to vessel 2 through pipe 14 provided with valve 15, the rate of flow being controlled and correlated with the proportion of solvent in the bath so that the liquid introduced from vessel 13 serves to compensate for the precipitant and solvent carried from the bath by the freshly formed fibers. In this way, the relative proportions of the precipitant and solvent in the setting bath are maintained substantially constant.

Vessel 2 is provided with an overflow pipe 16 for maintaining the level of the setting bath constant, and a vertically adjustable overflow pipe 17 associated with vessel 13 permits withdrawal of any liquid from the washing step which is not delivered to vessel 2. The withdrawn liquid may be stored for later use as a setting bath.

When the spinning is conducted at room temperature, as is preferred, or at temperatures below 100° C., and the washing liquid is heated, it is necessary to cool the liquid from the washing step before delivering it to the bath. This may be accomplished by associating any suitable cooling means, for example, a cooling coil 18, with vessel 13 as shown, through which a cooling fluid is circulated to adjust the temperature of the liquid collected in vessel 13 to the temperature of the spinning bath before it enters vessel 2.

An advantage of the present method is that the spinning solvent is recovered from mixtures in which it is present in relatively high concentration i. e., from the setting bath or from liquid remaining after initial washing of the fibers or the like.

If the washing liquid is a mixture of the precipitant and solvent, the proportion of solvent present therein must be controlled and should not be greater than one-half the amount of solvent present in the setting bath.

If it is desired to stretch the article for orientation, the article may be stretched prior to, during, or after the initial washing at temperatures depending on the material shaped, and may or may not be given an after-stretch. For example, freshly-formed fibers of the acrylonitrile polymers or blends may be stretched 100 to 300% at temperatures up to 100° C., or they may be stretched more than 300% at temperatures above 100° C., and such stretching may be the only stretch given the fibers. Or the fibers may be stretched up to 200 or 300% at temperatures of 100° C., and after-stretched at temperatures above 100° C., the after-stretching being performed either before or after final drying of the

fibers. In the embodiment illustrated on the drawing, the acrylonitrile polymer fibers may be stretched between the godets 4 and 7 simultaneously with washing thereof with water at any temperature up to 100° C., for instance a temperature between ordinary room temperature and 100° C., and then after-stretched at temperatures above 100° C. If the acrylonitrile polymer fibers are to be simultaneously stretched and heated to a temperature above 100° C., the godet stretch during washing may be omitted, or the stretch imparted to the fibers at temperatures up to 100° C. may be supplemented by an after-stretch at a temperature above 100° C.

As previously indicated, the invention may be used in the production of shaped articles, especially fibers of the acrylonitrile polymers, which term is intended to include polyacrylonitrile, copolymers and interpolymers of acrylonitrile with one or more other vinyl-type monomers containing at least 70% of acrylonitrile by weight in the polymer molecule, and blends comprising the acrylonitrile polymers. Examples of the latter are those compositions obtained by blending an acrylonitrile polymer containing, by weight in the molecule at least 70% of acrylonitrile with a copolymer of from 10 to 70% of acrylonitrile and from 30 to 90% of a vinyl-substituted heterocyclic tertiary amine, such as a vinylpyridine, to obtain a blend having an overall content of the polymerized vinyl-substituted tertiary heterocyclic amine of from 2 to 50%, based on the weight of the blend.

The following examples illustrate a specific embodiment of the invention:

*Example I*

Using apparatus as shown in the drawing, a 3000 filament tow was formed by continuously extruding a spinning solution comprising a homogeneous mixture of N,N-dimethylacetamide and 14.2% by weight of a polymer containing about 95% of acrylonitrile and about 5% of 2-vinylpyridine through a spinneret into a setting bath at room temperature and consisting of 58% of N,N-dimethylacetamide and 42% of water, by weight, the solution being delivered through the spinneret at a rate of 1.76 lbs./minute. The tow of filaments carried 0.5 lb. of N,N-dimethylacetamide per minute out of the setting bath into the trough 6. Water at about 100° C. was delivered to the trough at a rate of a gallon (8.33 lbs.) per minute. The liquid from the washing was collected in vessel 13, in which it was cooled to room temperature. From vessel 13 the liquid was continuously delivered to the bath in vessel 2 at a rate of 0.146 gallon (1.21 lbs.) per minute. Under these conditions, the composition of the setting bath remained at 58% of N,N-dimethylacetamide and 42% of water from the beginning to the end of the spinning which was performed continuously over a period of eight hours.

*Example II*

Using apparatus as shown in the drawing, a 5000 filament tow was formed by continuously extruding a spinning solution comprising a homogeneous mixture of N,N-dimethylacetamide and 14.2% of a copolymer of 95% acrylonitrile and 5% of 2-vinylpyridine, at room temperature and consisting of 58% of N,N-dimethylacetamide and 42% of water, by weight, the solution being delivered through the spinneret at a rate of 2.937 lbs. per minute. The tow of filaments carried 0.834 lb. of N,N-dimethylacetamide per minute

from the setting bath into trough 6. Water at about 100° C. was delivered to the trough from vessel 9 at a rate of one gallon (8.33 lbs.) per minute. The water from the washing which consisted of water and 9.12% of N,N-dimethylacetamide, was collected in vessel 13, in which it was cooled to room temperature by the cooling fluid circulating in coil 18, and from which it was continuously delivered to the bath in vessel 2 at a rate of 0.26 gallon (2.17 lbs.) per minute. Under these conditions the composition of the setting bath was maintained at 58% of N,N-dimethylacetamide and 42% of water throughout the spinning, which consumed eight hours.

The apparatus and method illustrated are particularly advantageous in the production of acrylonitrile polymer yarns which are unique in that, as disclosed in the pending application of Howard M. Hoxie and Helen G. Sommar, Serial No. 83,374, filed, March 25, 1949, the amount of residual solvent present in the yarns is critical to the stretch which the yarns are capable of accepting at elevated temperatures. For some purposes, it may be desirable to reduce the residual spinning solvent in or on the acrylonitrile polymer yarns to less than 1.5% by weight before stretching the yarns at elevated temperatures, for optimum stretch and improvement in the tenacity at any given temperature from 100° C. up to the temperature at which the yarn is damaged. The yarn leaving the setting bath comprising the solvent and precipitant contains an amount of solvent which is appreciably greater than 1.5% by weight, and ordinarily, prolonged washing would be required to reduce the solvent to less than 1.5%. However, in practicing this invention, the conditions, such as the length and width of trough 6, the angle of inclination of the trough with respect to vessels 2 and 9, the rate of flow of the washing liquid through the trough countercurrently to the yarn advancing from the bath, and the temperature of the washing liquid may be selected so that the yarn leaving the trough after the initial washing contains less than 1.5% of the spinning solvent and additional washings are not necessary prior to stretching the yarns at temperatures above 100° C.

Since certain changes may be made in carrying out the invention without departing from its spirit and scope, it is intended that all matter contained in the foregoing description is to be interpreted as illustrative and not in a limiting sense. In the claims, the terms "solvent" and "solution" are intended to include true solvents and solutions as well as dispersing agents and dispersions or colloidal solutions or mixtures in which the fiber- or film-forming material is substantially uniformly dispersed. The term "fibers" is intended to include filaments and yarns.

I claim:

1. A method of forming artificial and synthetic fibers and other shaped articles which comprises continuously extruding a solution of the material to be shaped into a setting bath comprising a mixture of the solvent and a liquid precipitant for the material to be shaped, which precipitant is an extractive for the solvent, continuously withdrawing the shaped article from the setting bath to the atmosphere, continuously washing the article as it advances from the setting bath, and above the level of the setting bath, with a confined stream of liquid flowing countercurrently to the direction of travel of the article

and consisting of the precipitant and at most a minor proportion of the extrusion solvent, collecting the liquid from the washing step, and continuously delivering liquid collected from the washing step to the setting bath in a controlled amount which is dependent on the relative proportion of precipitant to solvent in the liquid from the washing step and on the amount of solvent introduced into the bath by extrusion of the solution of the material to be shaped, so that the relative proportions of precipitant and solvent in the setting bath are thereby maintained substantially constant from the beginning to the end of the extrusion.

2. A method as in claim 1, wherein the article is stretched simultaneously with washing thereof.

3. A method as in claim 1, wherein the material to be shaped comprises an acrylonitrile polymer containing, by weight in the polymer molecule, at least 70% of acrylonitrile.

4. A method as in claim 1, wherein the material to be shaped is a blend of an acrylonitrile polymer containing, by weight in the polymer molecule, at least 70% of acrylonitrile with a copolymer of from 10 to 70% of acrylonitrile and from 30 to 90% of a vinyl-substituted heterocyclic tertiary amine.

5. A method as in claim 1, wherein the material to be shaped is a blend of an acrylonitrile polymer containing, by weight in the polymer molecule, at least 70% of acrylonitrile and a copolymer of from 10 to 70% of acrylonitrile and from 30 to 90% of a vinylpyridine.

6. A method as in claim 1, wherein the material to be shaped is a cellulose organic acid ester.

7. A method as in claim 1, wherein the material to be shaped is secondary cellulose acetate.

8. A method as in claim 1, wherein the material to be shaped is a synthetic resin.

9. A method of forming synthetic fibers from a fiber-forming composition comprising an acrylonitrile polymer containing, by weight in the polymer molecule, at least 70% of acrylonitrile, which comprises continuously extruding a solution of the polymer in dimethylacetamide into a setting bath comprising a mixture of water and dimethylacetamide in a selected proportion between 20

and 70% by volume, continuously withdrawing the fibers from the bath to the atmosphere, continuously washing the fibers advancing from the bath, and above the level of the bath, with a confined stream of liquid consisting of water and at most a minor proportion of dimethylacetamide flowing countercurrently to the direction of travel of the fibers, collecting the liquid from the washing step, and continuously delivering liquid collected from the washing step to the setting bath in a controlled amount which is dependent on the relative proportion of water to dimethylacetamide in the liquid from the washing step and on the amount of dimethylacetamide introduced into the bath by the solution of the polymer, so that the relative proportions of water and dimethylacetamide in the setting bath are thereby maintained substantially constant from the beginning to the end of the extrusion.

10. A method as in claim 9, wherein the fibers advancing from the setting bath are washed with water having a temperature between room temperature and 100° C.

11. A method as in claim 9, wherein the fibers are stretched simultaneously with washing thereof.

12. A method as in claim 9, wherein the fibers advancing from the setting bath are washed at a temperature between room temperature and 100° C., and stretched simultaneously with washing thereof.

13. A method as in claim 9, wherein the material to be shaped is a blend of an acrylonitrile polymer containing, by weight in the polymer molecule, at least 70% of acrylonitrile, with a copolymer of from 10 to 70% of acrylonitrile and from 30 to 90% of a vinyl-substituted heterocyclic tertiary amine.

14. A method as in claim 9, wherein the material to be shaped is a blend of an acrylonitrile polymer containing, by weight in the polymer molecule, at least 70% of acrylonitrile, with a copolymer of from 10 to 70% of acrylonitrile and from 30 to 90% of a vinylpyridine.

HOWARD M. HOXIE.

No references cited.